# EUROPEAN PATENT SPECIFICATION

(11) **EP 0 049 260 B1**
(45) Date of publication and mention of the grant of the patent: **02.05.1984**
(21) Application number: 81900934.1
(22) Date of filing: 15.04.1981
(51) Int. Cl.: E01C 7/32, C09J 3/30, C09J 5/06

(54) **PROCESS FOR TACK COATING IN ROAD SURFACING**
VERFAHREN ZUM AUFBRINGEN EINER HAFTSCHICHT AUF STRASSENOBERFLÄCHEN
PROCEDE D'APPRET POUR LE REVETEMENT D'UNE ROUTE

(30) Priority: 17.04.1980 SE 8002888
(43) Date of publication of application: 14.04.1982
(73) Proprietor: AB SKANSKA CEMENTGJUTERIET, S-201 10 Malmö (SE)
(72) Inventor: CHRISTENSEN, Ib Finn Robert, S-237 00 Bjärred (SE)
(74) Representative: Rosenquist, Holger
(86) International application number: SE8100117
(87) International publication number: WO8103039

## Description

The present invention relates to a process for tack coating between layers of road surfacing material such as asphalt concrete where an existing layer is swept clean and sprayed with a thin film of asphalt tack coat, whereafter asphalt is layed out on top of the tack coat.

A road surface is built up layer after layer with different materials for the various functions of the road. In order to assure that no slippage occurs between the layers, it is necessary to bind the layers with a thin tack coat. Normally the tack coat is only laid between the uppermost asphalt layers and not between the gravel layers which have by themselves sufficient friction between them.

The tack coat normally consists of an asphalt which has been dissolved in a solvent, e.g. naphta, or of an asphalt which has been emulsified in water. In the former case one speaks of an asphalt solution, and in the latter case of an asphalt emulsion. The asphalt solution is however of less interest now and will presumably disappear completely from the market because of the fact that it contains solvents which can be used for other purposes, i.e. as motor fuels, and the fact that they create a hazardous working environment.

In conventional tack coating, the tack coat is. left to dry, and the water evaporates, leaving a sticky film of asphalt. This process is quite disadvantageous, since a special work team and a separate unit are required for the tack coating plus the fact that a waiting period is required for drying.

The purpose of the present invention is to achieve a process for tack coating between layers of surfacing material, which does not have the above-mentioned disadvantages, which provides full adhesive effect immediately and which provides better adhesion than conventional tack coating.

This is achieved by means of the process according to the present invention, which is characterized in that the asphalt compound is laid out immediately after the existing asphalt concrete layer has been cleaned and tack coated, and in that the tack coat is dried and broken by the applied fresh and hot asphalt compound.

According to a preferred embodiment of the invention, an aqueous emulsion of an asphalt is used as the tack coat.

Further characteristics and advantages of the present invention will be revealed in the following detailed description.

Asphalt compound, which consists of gravel and asphalt, is made in asphalt plants. From there, the asphalt is driven in trucks to the surfacing site and is dumped into an asphalt laying machine or is laid out manually. The asphalt compound then has a temperature of about 150°C. After this compound has been applied and rolled, it is called asphalt concrete.

In order to avoid slippage between the asphalt concrete layers, a tack coat is used, as was mentioned above, the composition of which is specified in construction standards.

According to the technique which is the only one used at present, the existing asphalt concrete layer is first brushed clean, whereafter the tack coat is spread out by a separate work team with a special separate unit. Then one waits about 1/4 to 3 hours until the water or solvent has evaporated, leaving a thick, sticky asphalt film. Only then is the asphalt compound for the next layer laid out and rolled.

This binding method only produces an adhesion on the "tops", i.e. a surface adhesion.

The reason for waiting until the water has evaporated is that according to prevailing wisdom up to now, full adhesive effect is not achieved immediately, and this is necessary to prevent the new layer from slipping during the subsequent rolling and under traffic loads.

Tests have now shown that it is not necessary to allow the tack coat to dry. Rather, in complete contrast to previous wisdom, a better result is obtained if the tack coat is now allowed to dry prior to application of the asphalt compound.

According to the invention, the fresh, hot asphalt compound is applied immediately after the sweeping and the spreading of the tack coat, so that the asphalt compound drops on the wet tack coat film.

The tack coat is spread in amounts on the order of 0.2-0.4 kg per square meter and has a water content of about 30-50 per cent. This should be compared with the asphalt compound, which has a temperature of about 150°C and which is laid in amounts of about 60-120 kg per square meter.

When the hot asphalt is laid on the tack coat, the water in the tack coat or tack coat emulsion will boil violently and be vaporized, thus breaking the emulsion. This conversion results in a sharp increase in volume in the tack coat and appears as foam. The foaming and increased pressure forces the adhesive into the pores and capillaries both upwards and downwards, producing especially good adhesion at full effect immediately. A deep-acting adhesion is obtained which is clearly superior to the adhesion obtained by conventional tack coating.

Any remaining water in the pores etc. does not affect the adhesive result, which is best demonstrated by the fact that water-coated rollers can be used to avoid having the newly laid asphalt compound stick to the rollers, without resulting in any negative effects.

Series of tests carried out on a pilot scale to determine whether the method would work, have shown that significantly better results as regards the mechanical adhesion are obtained than with the conventional technique, and, as was indicated above, this depends on, among other things, the deep-acting ahesive effect, which is obtained by the increase in volume of the tack coat as the water is vaporized.

The advantages of the process according to the invention are thus that the need for an extra work team for the tack coating work is eliminated, as well as the need for a separate task coating unit.

Furthermore, the waiting time for breaking and drying of the tack coat is eliminated, resulting in a considerable time savings in the road servicing work. At the same time, an improved mechanical adhesion is obtained between the layers.

The process according to the invention is most suited to tack coats in the form of an aqueous emulsion, but will work for all asphalt binders which are used at present if the amounts of tack coat are adapted to the process.

## Claims

1. Process for tack coating between layers of road surfacing material, such as asphalt concrete, where an existing layer is swept clean and spread with a thin film of asphalt binder or tack coat, whereafter asphalt compound is laid out on the tack coat, characterized in that the asphalt compound is laid out immediately after the existing asphalt concrete layer has been swept clean and tack coated, and in that the tack coat is dried and broken by the applied fresh, hot asphalt compound.

2. Process according to claim 1, characterized in that an aqueous emulsion of an asphalt is used as a tack coat.

3. Process according to claims 1-2, characterized in that the asphalt compound with a temperature of about 150°C is applied onto the tack coat, thereby vaporizing the water in the tack coat in order to achieve such an increase in volume in the tack coat that it penetrates into pores and capillaries in the two layers, thereby achieving a deep adhesion.

## Patentansprüche

1. Verfahren zum Kleben zwischen Schichten aus Strassendeckenmaterial, wie Asphaltbeton, wo eine vorhandene Schicht ausgekehrt und mit einem dünnen Film aus Asphaltklebstoff oder Klebstoff bespritzt wird, wonach die Asphaltmasse auf den Klebstoff ausgebreitet wird, dadurch, gekennzeichnet, dass die Asphaltmasse unmittelbar nach dem Auskehren und Kleben der vorhandenen Asphaltbetonschicht ausgebreitet und der Klebstoff getrocknet und von der aufgelegten frischen und heissen Asphaltmasse gebrochen wird.

2. Verfahren nach Anspruch 1, dadurch, gekennzeichnet, dass als Klebstoff eine wässrige Emulsion eines Asphalts verwendet wird.

3. Verfahren nach Anspruch 1-2, dadurch gekennzeichnet, dass die Asphaltmasse mit einer Temperatur von etwa 150°C auf den Klebstoff aufgelegt wird, wodurch das Wasser im Klebstoff verdampft wird, um eine solche Volumenvermehrung des Klebstoffes herbeizuführen, dass dieser in die Poren und Kapillaren der beiden Schichten eindringt und ein tiefgehendes Kleben bewirkt.

## Revendications

1. Procédé de collage entre des couches de matière de revêtement routier, comme du béton d'asphalte, dans lequel une couche existante est balayée et arrosée par projection d'une pellicule fine de colle d'asphalte ou d'adhésif, après quoi une pâte d'asphalte est étalée sur la colle, caractérisé en ce que la pâte d'asphalte est étalée immédiatement après le balayage et le collage de la présente couche en béton d'asphalte et en ce que la colle est séchée et se coupe par la pâte appliquée qui est fraîche et chaude.

2. Procédé selon la revendication 1, caractérisé en ce que l'on utilise à titre de colle une émulsion acqueuse d'un asphalte.

3. Procédé selon la revendication 1 à 2, caractérisé en ce qu'une pâte d'asphalte ayant une température d'environ 150°C est appliquée sur la colle, au moyen de quoi l'eau contenue dans la colle est vaporisée afin de provoquer une telle augmentation de volume de la colle que celle-ci pénètre dans les pores et les capillaires des deux couches produisant ainsi une adhésion en profondeur.
